

June 3, 1930.

J. D. JONES

1,761,672

MANUFACTURE OF RAILS AND TIE PLATES

Filed Dec. 7, 1926

2 Sheets-Sheet 1



June 3, 1930.

J. D. JONES

1,761,672

MANUFACTURE OF RAILS AND TIE PLATES

Filed Dec. 7, 1926

2 Sheets-Sheet 2



## UNITED STATES PATENT OFFICE

JAMES D. JONES, OF SAULT STE. MARIE, ONTARIO, CANADA, ASSIGNOR TO EMIL GATHMANN, OF BALTIMORE, MARYLAND

## MANUFACTURE OF RAILS AND TIE PLATES

Application filed December 7, 1926. Serial No. 153,066.

This invention relates to the manufacture of rails and tie plates for railways, and the object of my invention is to produce such rails and tie plates from steel ingots in such an improved manner that the rails shall be of suitable quality steel—physically sound and of substantially uniform chemical composition, thus possessing the greatest possible strength and durability, and that the tie plates are physically sound and but so slightly segregated per unit plate as to in no way impair their strength and durability.

My method of procedure involves the use of steel ingots made by the most approved methods, in which molten steel is poured into ingot molds best adapted to produce an ingot which contains a relatively small percentage of physically unsound metal and only a small percentage of highly segregated steel definitely located near the top end of the finished ingot. An ingot having these characteristics is by my invention rolled into a bloom of desired length, the physically unsound or piped end of the bloom is cut off and discarded for remelting, and the remainder of the bloom is cut or divided in such manner that those portions of the bloom which are both physically sound and of substantially uniform chemical composition may be formed into rails, while that portion, which although physically sound contains a percentage which is usually excessively segregated, is further divided in such manner as to separate that portion of the bloom which is physically sound and substantially homogeneous from the part containing a degree of segregation which would be harmful to strength and reliability if used in rails.

The manner of making rails and tie plates according to my invention is illustrated in the accompanying drawings, which are largely diagrammatic. While these drawings illustrate one approved way of operating my invention, it will be understood that the process of operation may be varied to some extent.

Figure 1 shows a central vertical section of a steel ingot made in a Gathmann ingot mold, the percentages of physically sound and substantially homogeneous steel, of the sound but higher segregated steel and of the physically

unsound steel being indicated at various points.

Figure 2 shows on a smaller scale a steel ingot of the kind shown in Figure 1.

Figure 3 illustrates how the ingot shown in Figure 2 is rolled into a bloom.

Figure 4 illustrates how the unsound portion of the ingot is cut off after having been reduced to a bloom.

Figure 4A shows the unsound, cropped end of the bloom.

Figure 5 shows how the physically sound portion of the bloom is divided into sections, two of which sections are of steel which is physically sound and substantially homogeneous throughout and one of which sections while physically sound throughout contains a portion which is chemically segregated to such an extent as to be harmful or dangerous for use in rails.

Figure 6 illustrates how the three sections of the bloom are reheated.

Figure 7 illustrates how the physically sound and homogeneous sections of the bloom are rolled into rails.

Figure 7A illustrates the shape of the bloom after passing the first set of rolls.

Figure 7B shows the usual type of rail produced by other passes.

Figure 8 shows how the third section of the bloom is divided to separate the physically sound and homogeneous portion thereof from the remaining excessively segregated portion.

Figure 9 illustrates the manner of rolling that part of the bloom containing a high degree of segregation into tie plates.

Figure 9A shows the shape of the bloom resulting from the first passes.

Figure 9B shows the shape of the channel or blank obtained by subsequent passes, from which the tie plates are made.

Figure 10 is a perspective view of a form of finished tie plate.

As is now well-known to those familiar with the art, the first essential in the production of high quality steel for the manufacture of rails or other articles subject to heavy stresses is that the molten steel in the bath shall be cleansed as thoroughly as practicable from oxides and slag inclusions. The

steel, being of the required analysis, is cast in suitable ingot molds which, for convenience and economy of operation, should be of uniform size and shape. With molds of the Gathmann or big-end-and-up type and by proper finishing of the steel, it has been found possible to obtain ingots having a physically sound structure of from 90% to 95% of their weight. The physically unsound portion being definitely located at the uppermost part of the ingot and due to the shape and construction of the mold and refractory top, there is assurance of a definitely large percentage of the solidified ingot being physically sound.

Physical soundness is, however, not the only index of quality. As is well-known, steel during solidification is subject to segregation of various of its constituents, specifically carbon, sulphur and phosphorous, as well as any remaining products of oxidation, which lack of uniformity tends to reduce the strength and reliability of the products made from such ingots. Segregation is most pronounced in that portion of the ingot which is the last to solidify. In the use of the Gathmann type of mold, or big-end-up mold, solidification occurs progressively from the bottom to the uppermost portion of the ingot, while in the big-end-down mold the last of the steel to solidify is located at the central or even the lower portion of the ingot. It has been found that the chief zone of segregation lies from 3% to 4% below any visible physically defective portion of the ingot. A steel of .70 carbon ladle analysis frequently shows in the solidified ingot immediately below the physically flawed section a carbon content of .90 or more. The steel with the higher carbon content being physically sound is suitable for use in the manufacture of various articles such as tie plates for railways. It would not, however, be safe to make rails from steel containing widely varying degrees of carbon, as the strength and durability of the rail at various points would vary and the rail would not without injury stand the usual stresses to which it is subjected. Tie plates usually weigh from 10 to 40 pounds each and it is practically impossible for any great amount of segregation to occur in such articles, which are relatively small as compared with rails, which for example weigh from 700 to 2000 pounds each with a unit length of 39 feet, wherein excessive segregation might occur to a dangerous extent if rolled from a segregated portion of an ingot.

The ingots are preferably cast of uniform standard weight and length irrespective of the unit weights of rails to be rolled therefrom, i. e., if the ingot weight is established at 8000 pounds, six rails weighing 1000 pounds each would give a rail yield of 75% and a tie plate yield of 15%, while eight rails weighing 800 pounds each would give a rail yield of 80% and a tie plate yield of 10%, the ingot in both cases giving a sound product of 94%, of which 4% is lost due to unavoidable scaling and butt crop loss, of 3% and 1% respectively. In the 1000 pound rails approximately 10% of the tie plate steel would be fit for use in rail steel, but this would give a rail of under weight or short rail section not desired by the railroads; hence a high percentage of steel suitable for rails goes into tie plate. In the 800 pound rail only 5% of the rail-quality steel is used in the tie plate and in a still lighter rail, say of 750 pound section, 84% can be rolled into unit rails and only 1% of rail-quality steel is used in the tie plate.

As before stated, my object is to produce rails and tie plates which are not only physically sound but which are of substantially uniform chemical composition per unit weight.

Briefly stated, in carrying out my invention I use a Gathmann type big-end-up ingot. I crop and discard the physically unsound upper portion thereof, utilize the physically sound but partially segregated part of the ingot for making tie plates and most of the remaining physically sound and homogeneous parts of the ingot for making rails.

By a tie plate, it is to be understood, I mean a plate which is adapted to be secured to the wooden ties or sleepers used in the road bed of a railway and by means of which plate the rail base is indirectly supported on the ties.

It has been found desirable to employ tie plates made of physically sound metal, as otherwise the varying stresses due to traffic would soon enlarge any physical defect or flaw, which would lead to the breakage or disintegration of a physically unsound plate long before one made of a physically sound metal would wear out. Tie plates should be made of high carbon steel, preferably of the same analysis as the rails, as longer wear and less liability to deformation under pressure of both tie plate and rail is thus assured.

I have found it advantageous to employ an analysis of .65 to .75 carbon and .25 to .50 nickel in the production of rail and tie plate steel, as steel of such structure not only has a high resistance to deformation but also is substantially rust proof.

Referring now to the drawings, the ingot I shown in Figure 1 should be made of well de-gasified steel formed in a big-end-up mold of the Gathmann type. The ingot is made from steel which, analyzed in the ladle, contains about .71 carbon, and the segregation of the carbon content is indicated at various points within the ingot by the letter C preceded by numerals indicating the percentage of carbon at the various levels.

It will be noted that the greatest concentration of segregation is found several per-

cent below the bottom of the pipe or shrinkage cavity P, or in the region containing the steel last to solidify. In Figure 1 the pipe extends only 5% to 8% from the top or upper 5 end of the ingot, and the highest segregation of carbon (.99 C.) extends several percent below the base of the pipe. The approximate percent of first grade steel, or that which can safely be used in the production of 10 rails, is graphically shown in Figure 1 by legends and figures placed thereon, the total amount of sound steel being approximately 92% to 95% in the ingot shown. As before stated, segregation extends somewhat below 15 the base of the pipe. The ingot shown in Figure 1 is relatively sound and homogeneous for as much as 85% from its bottom or base portion upwards.

For reducing the ingot to a bloom it is 20 passed through rolls in the manner diagrammatically indicated in Figure 3. As there shown, a portion of the bloom is of physically sound and homogeneous steel. Another portion is of physically sound steel but 25 is segregated, and a third portion is of piped or unsound steel.

Figure 4 indicates diagrammatically a bloom reduced to the desired length, which for purposes of illustration may be considered 30 70 feet in length. About four feet of this bloom is unsound and is cropped in the manner illustrated in Figures 4 and 4A. The remaining portion of the bloom may then be divided into three parts or sections, 35 A, B and C, each twenty-two feet in length. The parts A and B are of physically sound and homogeneous steel. The part C has a portion y of sound homogeneous steel, and a portion x which is sound but segregated. 40 The parts A and B are suitable for making rails, and the parts y of the section C is suitable for making rails, while the part x is suitable for making tie plates.

The bloom is cut into lengths at the points 45 indicated, and the three bloom sections are reheated in a furnace F, of suitable construction, in the manner illustrated in the plan view, Figure 6.

After the bloom sections A and B are thus 50 heated, they are preferably given roughing passes in a three-high mill and are rolled into rails in the manner illustrated in Figures 7, 7A and 7B.

The bloom section C is passed to a shearing 55 press (Figure 8) either before or after being subjected to the roughing passes. Preferably it is given one or two passes before the parts x and y are separated by the shears in the manner indicated. The part y may be 60 rolled into rails in the manner before explained, but the part x is passed directly and without reheating to a mill where it is rolled into tie plate shapes as shown.

As before stated, I employ the usual method 65 of rolling rails, except that when the bloom

made from the top portion of the ingot has been reheated and preferably after it has an initial pass in the rolling mill it is brought to a shearing press and the excessively segregated portion (approximately 10% to 15% depending upon the weight of rail being rolled) is cut off. The segregated part x of the bloom is at once diverted and fed to an adjoining tie plate mill, without the necessity of again reheating, and rolled into tie plate shapes, while the part y is continued in the 70 75 passes of the rail mill until it has been shaped to the desired rail section.

By this method of manufacture I obtain a yield of from 90% to 95% of high grade 80 products, whereas from the old type of ingot and method of manufacture it is impossible to obtain a yield of more than 70% to 75% of the weight of the ingot in salable rail product. Not only is the percentage of commercial products greatly increased, but the rail and tie plate thus obtained are far superior in wearing qualities and reliability 85 to those produced by other methods heretofore employed.

I claim as my invention:

1. The method herein described of producing rails and tie plates from ingots containing less than 10% by weight of physically unsound structure and less than 25% by weight of relatively highly segregated structure, which consists in discarding and scrapping the physically unsound portion of the bloom and rolling that portion of the bloom which is physically sound but relatively highly segregated into relatively small tie plates and rolling that portion of the bloom which is both physically sound and substantially chemically homogeneous into rails.

2. The method herein described of producing rails and tie plates from ingots containing less than 10% by weight of physically unsound structure and less than 25% by weight of relatively highly segregated structure, which consists in discarding and scrapping the physically unsound portion of the bloom and rolling that portion of the bloom which is physically sound but relatively highly segregated into relatively small tie plates and rolling that portion of the bloom which is both physically sound and substantially chemically homogeneous into rails without reheating the bloom in the formation of tie plates.

In testimony whereof, I have hereunto subscribed my name.

JAMES D. JONES.